



US006440319B1

(12) **United States Patent**  
Meikle et al.

(10) **Patent No.:** US 6,440,319 B1  
(45) **Date of Patent:** Aug. 27, 2002

(54) **METHOD AND APPARATUS FOR PREDICTING PROCESS CHARACTERISTICS OF POLYURETHANE PADS**

(75) Inventors: **Scott G. Meikle; Guy F. Hudson**, both of Boise, ID (US)

(73) Assignee: **Micron Technology, Inc.**, Boise, ID (US)

(\*) Notice: Subject to any disclaimer, the term of this patent is extended or adjusted under 35 U.S.C. 154(b) by 25 days.

(21) Appl. No.: **09/641,165**

(22) Filed: **Aug. 16, 2000**

**Related U.S. Application Data**

(62) Division of application No. 08/914,994, filed on Aug. 20, 1997, now Pat. No. 6,114,706, which is a division of application No. 08/386,023, filed on Feb. 9, 1995, now Pat. No. 5,698,455.

(51) **Int. Cl.** <sup>7</sup> ..... **B44C 1/22**

(52) **U.S. Cl.** ..... **216/32; 51/306; 378/44;**

437/8

(58) **Field of Search** ..... 378/44; 437/8; 51/306; 216/34

(56) **References Cited**

**U.S. PATENT DOCUMENTS**

5,036,015 A \* 7/1991 Sandhu et al. ..... 437/8

5,256,880 A 10/1993 Loree et al. ..... 250/461.1  
5,483,568 A \* 1/1996 Yano et al. ..... 378/44  
5,698,455 A 12/1997 Meikle et al. ..... 438/8

**OTHER PUBLICATIONS**

Gutsche, Henry W.; Moody, Jerry W., *Journal of Electrochemical Society*, 125(1), 136-8, 1978.

\* cited by examiner

*Primary Examiner*—Anita Alanko

(74) *Attorney, Agent, or Firm*—Dorsey & Whitney LLP

(57) **ABSTRACT**

A measurement of polyurethane pad characteristics is used to predict performance characteristics of polyurethane pads used for chemical mechanical planarization (CMP) of semiconductor wafers, and to adjust process parameters for manufacturing polyurethane pads. In-situ fluorescence measurements of a pad that has been exposed to a high pH and high temperature environment are performed. The fluorescence characteristics of the pad are used to predict the rate of planarization of a wafer. A portion of one pad from a manufacturing lot is soaked in an organic solvent which causes the portion to swell. The relative increase in size is indicative of the performance characteristics of pads within the manufacturing lot. Statistical Process Control methods are used to optimize the CMP pad manufacturing process. Predicted pad characteristics are available for each pad.

**1 Claim, 4 Drawing Sheets**





FIG. 1



FIG. 2



FIG. 3



FIG. 4

**METHOD AND APPARATUS FOR  
PREDICTING PROCESS  
CHARACTERISTICS OF POLYURETHANE  
PADS**

**CROSS-REFERENCE TO RELATED  
APPLICATION**

This application is a divisional of pending U.S. patent application Ser. No. 08/914,994, filed Aug. 20, 1997 now U.S. Pat. No. 6,114,706, which is a divisional of 08/386,023 filed Feb. 9, 1995 and issued Dec. 16, 1997 as U.S. Pat. No. 5,698,455.

**FIELD OF THE INVENTION**

This invention relates to the use of chemical mechanical planarization (CMP) in the manufacture of semiconductor integrated circuits and more particularly to prediction of performance characteristics of polyurethane pads used for CMP of semiconductor wafers.

**BACKGROUND OF THE INVENTION**

During fabrication of integrated circuits, it is often desirable to planarize and/or polish the surface of a semiconductor wafer. One method of performing these tasks is referred to as chemical mechanical planarization (CMP). In general, the CMP process involves rotation or random movement of a wafer on a polishing pad in the presence of a polishing slurry. The polishing pad is typically formed of a polyurethane material.

Downward pressure on the wafer against the pad, rotational speed of the wafer and the pad, slurry content and pad characteristics determine the rate at which material is removed from the surface of the wafer, and the uniformity of the resulting wafer surface.

Determination of how long a wafer should be planarized or polished has proven to be a difficult task. An apparatus and method for in-situ measurement of the thickness of a material to be planarized for CMP end point determination is described in U.S. Pat. No. Re. 34,425 to Schultz.

Methods of controlling the pressure exerted on the wafer against the pad, rotational speed or random movement of the wafer on the pad and slurry composition are well known in the art. Condition and performance characteristics of the polyurethane pad are more difficult to determine. The ability of a pad to planarize the surface of a wafer varies substantially from pad to pad and over the life of an individual pad.

After a wafer has been through the CMP process the pad will be conditioned to prepare it for another wafer. The conditioning process comprises a controlled abrasion of the polishing pad surface for the purpose of returning the pad to a state where it can sustain polishing. The ability of the conditioning process to return the pad to a state where it can efficiently planarize an additional wafer is dependent upon the pad itself and the conditioning parameters. After planarizing several hundred wafers, the pad may no longer be useful for planarizing wafers despite the conditioning process.

The ability to predict performance characteristics of new and used polyurethane pads would be a great benefit to users and manufacturers of such pads.

**SUMMARY OF THE INVENTION**

A measurement of chemical bonding of polymer chains within a polyurethane pad manufactured for chemical

mechanical planarization (CMP) of semiconductor wafers is used to predict performance characteristics of the pad, and to adjust process parameters for the subsequent manufacture of additional polyurethane pads.

5 After manufacturing a lot, one pad or a portion of a pad from the manufacturing lot is soaked in an organic solvent which causes the pad material to swell. It is believed that the relative increase in size is indicative of chemical bonding of polymer chains within the pad. The increase in pad size is 10 indicative of the performance characteristics of the pad. Statistical Process Control methods are used to optimize the pad manufacturing process. A manufacturing lot may consist of any number of pads which are deemed to have been manufactured under conditions which tend to cause all pads 15 within the lot to have very similar performance characteristics. Measurements of pad performance predictors allow predicted pad characteristics to be available for each pad. The predicted performance characteristics may be used as a measure of quality of the pad, and may also be provided to 20 pad end users.

Pad characteristic measurements may be taken before any wafers are planarized. Measurements may also be taken after each wafer is planarized or at intervals throughout the life of the pad. Repeated use of the pad impacts the polishing/ 25 planarizing ability of the pad. During the CMP process, polyurethane pads are often exposed to high pH (9.0 to 13.0) and high temperature (0 to 90 C.) environments. A correlation 30 between fluorescence characteristics and pad performance has been noted in pads that have been exposed to such conditions. In order to predict future performance of a used pad, in-situ fluorescence measurements of the pad are performed. The fluorescence characteristics of the pad are 35 also believed to be indicative of the chemical bonding of polymer chains within the pad, and are used to predict the effect conditioning will have on the pad. The predicted effect of conditioning is then used to predict performance characteristics of the pad. The measurement of pad fluorescence characteristics also allows for worn or substandard pads to be replaced prior to wafer processing.

**BRIEF DESCRIPTION OF THE DRAWINGS**

The features of the invention as well as objects and advantages will be best understood by reference to the 45 appended claims, detailed description of particular embodiments and accompanying drawings where:

FIG. 1 is a plot of fluorescence wavelength versus intensity for a CMP pad;

FIG. 2 is a plot of fluorescence wavelength peak divided 50 by 436 nanometers versus wafer material removal rate of a CMP pad;

FIG. 3 is a plot of pad swelling versus wafer material removal rate; and

FIG. 4 is a diagram of an apparatus for in-situ measurement 55 of the fluorescence characteristics of a CMP pad.

**DETAILED DESCRIPTION OF THE  
PREFERRED EMBODIMENTS**

60 FIG. 1 shows the fluorescence properties of a typical polyurethane CMP pad before (PRE) and after (POST) a five hour exposure to a pH 10.5 solution at a temperature of 60 C. After exposure, there is a shift in the spectra to shorter wavelengths. The amount of shift varies from pad to pad. 65 Two characteristic intensity peaks are noted in the spectra. One at approximately 436 nanometers and a second maximum peak at a wavelength which varies from pad to pad. In

a preferred embodiment of the invention, a pad is exposed to the high pH and high temperature environment prior to making the fluorescence measurement so that the measurement is made after the characteristic shift in wavelengths.

FIG. 2 shows a plot of maximum fluorescence intensity divided by the intensity at 436 nanometers versus the planarization rate of a semiconductor device wafer. This plot shows a relationship between the fluorescence characteristics of the CMP pad and the pad's ability to planarize a semiconductor wafer. The planarizing rate is also related to the process stability, defect density and uniformity of the processed wafer. Knowledge of the performance characteristics of the pad allows for substandard pads to be rejected prior to use, this in turn reduces the amount of wafer material needed to be scrapped.

FIG. 3 is a plot of the swelling of a portion of a CMP pad soaked in N-Methyl-2-pyrrolidone (NMP) for twenty-four hours versus the rate of planarization of a semiconductor device wafer which is planarized by the pad. Increases in swelling beyond twenty-four hours are not very large; however, longer or shorter periods of time may be used. The swelling measurement shown is a measurement of increase in pad area. The increase in pad volume, or simply the increase in length of a strip of pad material may also be used. Greater swelling indicates that the planarization rate will be lower. It is believed that other organic solvents such as MEK, MIBK, THF, Xylene and MeCl<sub>2</sub> may be used with similar results.

The plots of FIGS. 1, 2 and 3 show that measurements of polyurethane pad characteristics can be used to predict the planarization characteristics of the pad. The predicted planarization characteristics allow for a determination of planarization time in a CMP process. Predicted planarization characteristics of a CMP pad can also be used for process control and quality control in the manufacture of CMP pads. This data may be sent with the pads to CMP pad customers in the form of predicted planarization characteristics for particular CMP processes. The inventive method of mea-

suring pad characteristics may be used to perform incoming inspection on the pads. Substandard pads can be rejected before they are ever used.

FIG. 4 shows an in-situ method of measuring fluorescence characteristics of CMP pads in a CMP apparatus. A pad 10 is secured to a platen 20 which is rotateable. A radiation source 30 is secured above the pad surface. The radiation source may be a source of ultraviolet light which is directed at the pad. The wavelength of the source is preferably below 350 nanometers. Prior to and/or after conditioning, the radiation source is used to cause the pad to fluoresce. An electromagnetic radiation detection device, or photodetector, 40 is mounted above the pad surface. Emission from the pad is typically in the range of 200 nanometers to 800 nanometers.

A measure of intensity versus wavelength of electromagnetic radiation is used to determine when the pad should be replaced, and how the pad will perform when processing wafers. This prediction of pad performance is used to adjust the CMP process variables in order to achieve consistent CMP results with fewer end point detection measurement requirements.

While the present invention has been described with reference to specific preferred embodiments, alternate embodiments and modifications may be employed by persons skilled in the art without departing from the scope of the invention as defined by the following claims.

What is claimed is:

1. A method for manufacturing an integrated circuit, comprising:  
forming a layer of material on a wafer substrate; and  
polishing the wafer in a chemical mechanical planarization apparatus for a period of time dependent upon a measurement of chemical bonding of polymer chains within a pad attached to the chemical mechanical planarization apparatus.

\* \* \* \* \*